

# UNITED STATES PATENT OFFICE.

ERIK OLLESTAD, OF ST. PAUL, MINNESOTA, ASSIGNOR OF ONE-HALF TO  
ANDREW JENSON, OF SAME PLACE.

## TANNING PROCESS.

SPECIFICATION forming part of Letters Patent No. 401,715, dated April 16, 1889.

Application filed March 2, 1888. Serial No. 265,955. (No specimens.)

*To all whom it may concern:*

Be it known that I, ERIK OLLESTAD, a citizen of Norway, residing at St. Paul, in the county of Ramsey and State of Minnesota, have invented certain new and useful Improvements in the Process of Tanning Hides; and I do hereby declare the following to be a full, clear, and exact description of the invention, such as will enable others skilled in the art to 10 which it appertains to make and use the same.

This invention relates to an improved process of tanning; and it has for its object the production of a softer and finer leather and stronger in much shorter time than heretofore, as will be more fully hereinafter described, and then specifically defined by the claim.

The ordinary method of tanning by the use of bark has one objection—that of consuming 20 too long a time in the process of tanning. Certain chemicals have been used of late which have considerably shortened the time of tanning; but those that have been used heretofore have not been entirely successful 25 in producing as good results as from the old method of bark-tanning. In my method I not only accomplish as good results as from the bark process, but make leather a great deal stronger and more water-proof, as well as 30 softer and more pliable. I make use of both chemicals and extracts. By "extracts" I wish to be understood as covering any extracts that may be used for the purpose of tanning—such as the extract of hemlock-bark, the extract of 35 oak-bark, japonica, &c. I use the extracts also for the reason that by using both chemicals and extracts the leather by being tanned in this way obtains the same properties as leather tanned in the ordinary bark process, which 40 fact is of great importance to the subsequent preparation in dyeing of the leather. The chemicals I make use of are blue vitriol, bichromate of potash, alum, and sulphuric acid. Soaking, fleshing, and the removing of hair are 45 done in the usual way. Large hides for belting or for other purposes where unusual strength is required are taken after the hair and flesh have been removed and placed as they are in the liquor.

50 The proportions of the ingredients used are as follows: In tanning ten ordinary hides I

use from ten to fifteen barrels of water, forty pounds of tanning extract, twenty pounds of alum, ten pounds of blue vitriol, eight pounds of sulphuric acid, and one and one-fourth 55 pound of bichromate of potash. After the above-named chemicals and extracts have been thoroughly dissolved I take one-fourth part of the same and put in a vat, together with the necessary water, which is then 60 poured into the stuffing-wheel. This liquor is then heated to a temperature of from 75° to 80° Fahrenheit, after which the hides are placed in the liquor, and the stuffing-wheel is kept turning around about one hour at a 65 time three times per day. The third day the hides are taken out and another one-fourth part of the above-named solution is added to the liquor in the stuffing-wheel, which is then heated to a temperature of 70°. The 70 hides are again placed in the stuffing-wheel, which is kept turning around at intervals, as before, until it is apparent that the liquor has lost its strength, when the hides are again taken out, and the remaining one-half of the 75 solution is added to the liquor in the stuffing-wheel, which is also heated to a temperature of 70°, and after the hides have been replaced therein it is kept turning around at intervals, as before, until in the course of 80 about fourteen days the hides will be tanned. In the washing of the leather I make use of ordinary lye extracted from maple-wood ashes and rub it well with good boiled train-oil on the grain or hair side, and with three-fourths part train-oil and one-fourth part of 85 rosin, which is boiled together, on the flesh side. The leather is now rubbed well with the above-named mixtures, according to its thickness, and hung up until about one-half 90 dried, when it is taken down and stretched and hung up again until entirely dried. It is then taken down, rolled, and finished.

In tanning skins or upper-leather, kid, &c., all impurities must first be removed, which 95 is done in the ordinary way. I now make use of muriatic acid (the quantity being small, just sufficient to continue to make the tannic liquid sour) instead of sulphuric acid. The time absorbed in tanning, on account of 100 the skins being lighter, is also reduced from two to eight days. After the skins are tanned

and taken out of the liquor they are thoroughly rinsed and washed in lye. They are then rubbed with a boiled mixture of train-oil and tallow and hung up until about one-half dry, when they are taken down and the above-named mixture thoroughly worked into the skins and again hung up until entirely dry. The skins are now placed in lye that is heated to a temperature of 25°, and all the grease is then washed out until they are entirely clean. They are then stretched and smoothed and again hung up to dry, after which they are ready for dyeing.

Importance is attached to the use of the blue vitriol and bichromate of potash, as

these ingredients render the leather soft, fine, and strong.

What I claim as new is—

As an improvement in the art of tanning, the process described, which consists in treating the hides with a solution composed, essentially, of water-tanning extracts, blue vitriol, alum, bichromate of potash, and sulphuric acid, as set forth.

In testimony whereof I affix my signature in presence of two witnesses.

ERIK OLLESTAD.

Witnesses:

C. SCHNAITH,

JOHN W. SCHREINER.